

## UNITED STATES PATENT OFFICE

2,134,554

## LUBRICANT

Lloyd P. Grobel, Schenectady, N. Y., assignor to  
General Electric Company, a corporation of  
New York

No Drawing. Application September 12, 1936,  
Serial No. 100,542

5 Claims. (Cl. 87-9)

The present invention relates broadly to lubricants or lubricating compositions. More particularly, it relates to and has as a main object to improve the lubricating properties of hydrocarbon oil such, for example, as petroleum hydrocarbon lubricating oils. The desired result is attained by incorporating with a hydrocarbon oil a small amount of a member of the group consisting of benzaldehyde, salicylic (or salicyl) aldehyde and benzoic acid.

For a consideration of what I believe to be novel and my invention attention is directed to the following specification and the claims appended thereto.

15 It has been known heretofore that the lubricating power or capacity, that is, the film strength, of hydrocarbon oils such as petroleum lubricating oils may be improved by incorporating therein or commingling therewith certain modifying agents such, for instance, as free fatty acids, naturally occurring fatty oils, halogenated organic compounds (e. g., chlorinated esters of fatty acids, chloracetic acid, benzyl chloride, etc.), certain phosphorous compounds such as tricresyl phosphate, various sulfur-containing compounds, and so forth.

20 Although the addition of a fatty oil to a petroleum hydrocarbon lubricating oil produces a composition of somewhat improved film strength, such a lubricant is not always completely satisfactory in use since fatty oils tend to break down, especially at high temperatures with known disadvantages. Likewise, admixture of fatty acids with petroleum hydrocarbon oils is not always 25 practically effective in producing desired results. The high molecular weight saturated fatty acids show low film strengths, while those of low molecular weight, although they show higher film strengths, are corrosive to metal surfaces in the 30 presence of moisture; and the unsaturated fatty acids tend to oxidize in use, forming undesirable gummy oxidation products. Other substances, such as those hereinabove mentioned by way of 35 example, may be effective in producing lubricants of improved film strength, but many of such compositions, for example, those containing halogenated organic compounds, are objectionable in that they are corrosive to metal surfaces such as iron, steel and the like under certain 40 conditions, for instance, in the presence of moist air.

45 In accordance with the present invention, high film strength lubricating oil compositions non-corrosive to metal surfaces are provided by intimately mixing with a hydrocarbon oil, such as a petroleum lubricating oil, a small amount, for example, from about 0.01 to 2.0 per cent by weight, of an organic compound selected from the group consisting of benzaldehyde, salicylic 50 aldehyde and benzoic acid.

To test the film strength of lubricants produced by this invention, I have used a modified Almen extreme pressure lubricant testing machine. This device, which determines the pressure at which a lubricating oil will break down 5 to allow metal to metal contact, is fitted with  $\frac{1}{4}$  inch by  $\frac{1}{2}$  inch bearings made from cold-rolled steel rods. The bearings are split, each half carrying the total load, which is applied through a lever system by weights. The test 10 shaft is made of ground unhardened steel drill rod and is run at 100 revolutions per minute. The two half bearings are assembled in proper position and sufficient lubricant poured into the housing to submerge the bearing surfaces. The 15 machine is started at light load and the load increased at 10 second intervals, by the addition of weights, at the rate of about 2,000 pounds per square inch bearing pressure. The weights are applied until seizure of the test bearing occurs 20 or the capacity (45,300 pounds per square inch bearing pressure) of the machine is reached, or friction becomes sufficiently great to cause shearing of a brass pin in the driving couple. After the tests have been run, the test shafts are 25 examined for corrosion after remaining for several days in a closed vessel in a water-saturated atmosphere.

The results of the tests shown in Table I illustrate the greatly increased film strength 30 possessed by lubricating oil compositions produced in accordance with this invention as compared with the original mineral oil and with lubricants containing other addition agents:

| Table I                                                                                                                                    | 35     |
|--------------------------------------------------------------------------------------------------------------------------------------------|--------|
| Pounds per square inch<br>pressure on rubbing sur-<br>faces when seizure of<br>test bearing occurs                                         |        |
| Unmodified, that is, "straight" petroleum hydrocarbon lubricating oil having a Saybolt Universal viscosity at 100° F. of about 220 seconds | 40     |
| Same oil plus 1% by weight stearic acid                                                                                                    | 7,200  |
| Same oil plus 1% by weight oleic acid                                                                                                      | 7,200  |
| Same oil plus 1% by weight nitrotoluene                                                                                                    | 10,400 |
| Same oil plus 1% by weight benzyl alcohol                                                                                                  | 17,400 |
| Same oil plus 1% by weight benzyl alcohol                                                                                                  | 45     |
| Same oil plus 1% by weight salicylic aldehyde                                                                                              | 21,000 |
| Same oil plus 1% by weight benzaldehyde                                                                                                    | 38,000 |
| Same oil plus 1% by weight benzaldehyde                                                                                                    | 50     |
| Same oil plus 1% by weight benzoic acid                                                                                                    | 39,000 |
| Same oil plus 1% by weight benzoic acid                                                                                                    | 39,500 |

55 Examination of the test shafts for corrosion, after several days in a moist atmosphere, showed that none of the oil compositions containing the stated addition agents had a corrosive effect upon the metal surfaces. On the other hand, when samples composed of the same mineral oil and a small amount of chlorinated compounds, for 60

instance, 1% by weight chloracetic acid in one case and 1% by weight benzyl chloride in another, were prepared and tested, it was found that although such oil compositions had high film strength, that is, withstood a pressure on the rubbing surfaces of the order of about 40,000 pounds per square inch before seizure occurred, such lubricant had a corrosive effect upon the test shaft.

10 0 In practicing this invention only a small quantity of the addition agent is added to a hydrocarbon lubricant. Benzaldehyde, salicylic aldehyde or benzoic acid of a technical grade of purity may be used. The addition agent is well blended 15 with the hydrocarbon oil by any suitable means, after which the composition is ready for use as a lubricant.

15 20 The invention is not limited to the preparation of oil compositions of improved film strength by admixture of the addition agent with a hydrocarbon oil of any particular viscosity, or of other particular physical or chemical properties, but is applicable to all hydrocarbon lubricants, including greases, irrespective of viscosity or classification. Lubricating compositions of this invention may be employed at any and all points 25 throughout any type of engine or machine structure, either in the form of an oil or a grease, and may be applied in the same manner as heretofore 30 has been the common practice in the lubrication of machine structures. The compositions are especially adapted for use in lubricating rubbing surfaces operating at comparatively low speeds,

for example, in the lubrication of gears, pinions and the like.

What I claim as new and desire to secure by Letters Patent of the United States is:

1. A lubricating composition of high film 5 strength comprising hydrocarbon oil and an organic compound selected from the group consisting of benzaldehyde, salicylic aldehyde and benzoic acid in an amount sufficient to increase the film strength of the said oil. 10

2. A lubricating composition of high film strength comprising petroleum hydrocarbon oil having incorporated therewith from 0.01 to 2.0 per cent by weight of an organic compound selected from the group consisting of benzaldehyde, 15 salicylic aldehyde and benzoic acid.

3. A lubricating composition of high film strength consisting essentially of a petroleum hydrocarbon lubricating oil and benzaldehyde in an amount sufficient to increase the film strength 20 of the said oil.

4. A lubricating composition of high film strength consisting essentially of a petroleum hydrocarbon lubricating oil and salicylic aldehyde in an amount sufficient to increase the film 25 strength of the said oil.

5. A lubricating composition of high film strength consisting essentially of a petroleum hydrocarbon lubricating oil and benzoic acid in an amount sufficient to increase the film strength 30 of the said oil.

LLOYD P. GROBEL.